

March 21, 1939.

L. H. MATTES

2,151,220

BUILDING COVERING MATERIAL

Filed July 30, 1937

FIG. 1.



FIG. 2.



FIG. 3.



INVENTOR.

LEE H. MATTES.  
Ollock & Kwock

ATTORNEYS

## UNITED STATES PATENT OFFICE

2,151,220

## BUILDING COVERING MATERIAL

Lee H. Mattes, South Bend, Ind., assignor to  
 Mastic Asphalt Corporation, South Bend,  
 Ind., a corporation of Indiana

Application July 30, 1937, Serial No. 156,568

3 Claims. (Cl. 91—68)

This invention relates to building covering material, and particularly to siding and the like formed of composition board and coated with suitable weatherproofing material.

5 Building covering material of this type has heretofore been conventionally manufactured by simply coating a sheet of composition board of the desired size and shape with a thermo-plastic material, such as bituminous asphalt, and applying granular material, such as grit, to the plastic material, the same being so applied and/or contoured as to present an ornamental appearance, as of brick work, at the coated face. The thermo-plastic material adheres to the face of the composition board satisfactorily under ordinary conditions; but the adhesion sometimes proves inadequate under conditions of high temperatures, as for instance extreme summer heat or radiated heat from various possible external 10 or mechanical sources. Thus under such conditions, the adhesion is broken, and the coating tends to slide downwardly on the face of the composition board. Also, the composition board commonly employed is of the type which comprises small particles of cellulose material, with or without a binder, compressed into a compact rigid board. Such material is subject to peeling, particularly peeling of a thin layer adjacent the face which is coated. This is particularly true 15 where water reaches the composition board, as where a combination of heavy rain and high wind may drive water behind the lower ends of the lowermost covering units on a building. Peeling may also be caused or started by striking an edge of the board. It is, therefore, the primary object of this invention to construct a material of this character in a manner to minimize sliding of the coating and peeling of the board, particularly peeling of a thin layer adjacent the face of the board.

20 A further object is to provide a material of this character wherein a plurality of recesses are formed in the coated face of the composition board into which the coating material extends.

25 A further object is to provide a material of this character wherein portions of the board are impregnated with the coating material for a substantial portion of the thickness thereof to bond the material of the board.

In the drawing:

Fig. 1 is a perspective view of a unit of building covering material.

Fig. 2 is a face view of a unit of composition board preparatory to coating.

Fig. 3 is an enlarged fragmentary sectional view of the material.

Referring to the drawing, which illustrates the preferred embodiment of the invention, the numeral 10 designates a unit of building covering material having for its foundation a substantially rectangular sheet of any conventional rigid composition board 11 of substantial thickness. This board is preferably provided with the ship-lap undercut flanges 13 at two adjacent edges, and with the inset ship-lap flanges 14 at the other two edges. One face of the board 11 has a plurality of spaced recesses or depressions 15 of substantial depth formed therein by any suitable means. These depressions are preferably narrow as compared to their depth. The recessed face of the board is then coated with a layer 16 of suitable thermo-plastic water-proofing material which enters the recesses 15 to provide tongues or projections 17 imbedded in the board. The portions 18 of board 11 surrounding recesses 15 are impregnated with the coating material as illustrated by the shaded portions of Fig. 3. Over the plastic coating is spread a layer of colored grit 19 which is pressed partially 20 therein to provide a colored protecting surface.

The coated face of the material is suitably processed by any of the methods well known in the art, to give to the same the appearance of brick work, as by impressing the grooves 20 30 therein to simulate a mortar joint. If desired, grit of a different color than the main or body layer of grit 19 may be applied in the grooved portions to further increase the mortar joint simulation.

35 It will be seen that the provision of recesses 15 in board 11 permits the tongues or projections 17 of coating material to be formed at the same time the coating material is applied, said tongues being integral with the coating. The recesses 40 are commonly formed by means of impaling members projecting radially from the periphery of a pressure roll, and it will be seen that this tends to provide the recess with roughened walls. These roughened walls facilitate and enhance 45 the normal impregnation of the coating material in the body of the composition board around the opening. This serves, consequently, to provide a positive interlock between the coating projections and the composition board. The extent of the impregnation may be readily observed 50 when the material is forcibly intentionally peeled or is transversely severed adjacent one of the recesses. When the board is forcibly and intentionally peeled, which peeling occurs only a sub- 55

stantial distance from the coating in this construction, the peel is substantially contoured and naturally results in the formation of protuberances opposite the tongues 17 of coating material. Inasmuch as this contoured impregnation 18 requires any peeling which is intentionally or otherwise produced, to occur at an angle to the normal direction of peel in the vicinity of tongues 17, the construction has increased resistance to 10 peeling or splitting than does any conventional construction. The tongues 17 and contoured impregnation 18 of the coating material thus serve to greatly enhance the strength of the composition board with respect to its resistance to 15 splitting and peeling. Also, these features enhance and increase the weather-resisting qualities of the product and minimize possibility of displacement or sliding of the plastic coating on the board.

20 I claim:

1. Building covering material comprising a composition board which is subject to peeling when coated with flexible plastic material, said board having a plurality of spaced depressions 25 of substantially greater depth than width formed in one face thereof, and a plastic waterproof

coating adhering to said face, portions of said plastic filling said depressions to prevent said peeling.

2. Building covering material comprising a composition board which is subject to delamination when coated with a flexible layer of plastic material, said board having a plurality of spaced depressions in one face thereof, said depressions being of greater depth than width, a coating of waterproof plastic adhering to said face and filling said depressions to prevent said delamination, said plastic impregnating said board adjacent said recesses.

3. Building covering material comprising a rigid, substantially thick board of compressed 15 comminuted cellulose material which is subject to delamination when coated with a flexible layer of plastic material, said board having deep narrow recesses in one face thereof, the walls of said recesses being rough, and a coating of water- 20 proof plastic adhering to said face and filling said depressions to prevent said delamination, said plastic impregnating said board adjacent the walls of said recess.

LEE H. MATTES.

25